

## UNITED STATES PATENT OFFICE

LEWIS JAMES KEELER, OF CLEVELAND, OHIO, ASSIGNOR TO BERYLLIUM CORPORATION OF AMERICA, OF NEW YORK, N. Y., A CORPORATION OF NEW YORK

## PROCESS FOR THE PRODUCTION OF BERYLLIUM ALLOYS

No Drawing.

Application filed November 14, 1925. Serial No. 69,153.

This invention relates to a method of making alloys of beryllium. Hitherto, most alloys of beryllium with other metals have been made either by simultaneous reduction of the mixed oxides by means of carbon, or by the electrodeposition of beryllium into molten metal cathodes. The former of these methods is open to the objection not only that relatively small yields are obtained, but also that large amounts of the objectionable beryllium carbide are formed. The second method has been found to be generally inadequate because of the slight tendency of beryllium to alloy with metals generally even when liberated at their surfaces; and alloys made in this manner generally show far lower beryllium content than would be expected from the amounts of beryllium theoretically electrodeposited into the second metal.

I have found that by simultaneous precipitation of the beryllium and the metal to be alloyed therewith during the electrolysis of electrolyzable beryllium salts, such alloys can readily be made. As an electrolyte may be used the double fluoride of beryllium and a more electropositive material such as sodium. During the electrolysis a reducible compound of the other metal (in the form of its salt or oxide) is added to the bath, and, if necessary, a beryllium salt or oxide may also be added. The beryllium content can easily be regulated by changing the ratio of added metal in the form of its oxide or salt to beryllium in the form of its oxide or salt. Where, as in the case of metals low in the electromotive series, such as copper and silver, simultaneous deposition is difficult because of the far greater tendency of the other metal to precipitate first either by thermal or electrolytic deposition, I have found it possible to make alloys directly by alternate additions, during the electrolysis, of the second metal in the form of a salt or oxide, and also beryllium in the form of an electrolyzable salt, preferably a halide or oxide. In either simultaneous deposition or alternate deposition, the second metal, in the form of particles just liberated, performs the function of carrying down with it such beryllium glob-

ules or lamellæ as might otherwise rise to the surface and be reoxidized.

As one example of operation the following instance may be cited, the details not being intended as at all restrictive but rather indicative of what was found to occur in the particular run in question.

Sodium-beryllium fluoride of the approximate composition  $2\text{NaF} \cdot \text{BeF}_2$  was melted down in a graphite crucible held at  $1100^\circ$  to  $1200^\circ$  C. by means of external heating. A carbon rod one inch in diameter served as anode, the crucible acting as cathode.

The applied voltage varied from 5 to 8 volts, the current varying in turn from 150 to 300 amperes. At intervals additions of copper carbonate and beryllium oxide were made. The alloy was recovered by pouring off the supernatant salts and pouring the metal into a mold.

It will be understood that the addition of beryllium oxide is not essential even in the above cited example, since the double fluoride can itself be utilized as the source of beryllium. Similarly, any salt of copper decomposing either electrolytically or thermally to metallic copper under such conditions could have been used instead of the salt specified.

The method above described is generally applicable to the alloying of beryllium with one or more other metals.

I claim:

The method of producing alloys of beryllium which comprises subjecting a fused bath containing beryllium compound to electrolysis under conditions capable of precipitating metallic beryllium and alternately supplying to the bath a beryllium compound and a compound of an alloying metal, capable of liberating metallic beryllium and said alloying metal, respectively, under the conditions of the bath.

In testimony whereof, I affix my signature.

LEWIS JAMES KEELER.

95

100